

J.W. Jarboe.  
Molded Articles.  
No 92,611. Patented July 13, 1869.

Fig; 1;



Fig; 2;



Inventor:

J.W. Jarboe  
West Brownlowbridge  
Ohio

Witnesses:

Fred. Haynes  
McCrory

# United States Patent Office.

JOHN W. JARBOE, OF GREEN POINT, NEW YORK.

Letters Patent No. 92,611, dated July 13, 1869.

## IMPROVED COMPOSITION WAGON-BODY.

The Schedule referred to in these Letters Patent and making part of the same.

To all whom it may concern:

Be it known that I, JOHN W. JARBOE, of Green Point, in the county of Kings, and State of New York, have invented a new and useful Improvement in Wagon or other Vehicle-Bodies, of which the following is a full, clear, and exact description, reference being had to the accompanying drawing, forming part of this specification, and in which—

Figure 1 represents a view, in perspective, of a wagon-body constructed in accordance with my improvement, and

Figure 2, a longitudinal vertical section of the same.

Similar letters of reference indicate corresponding parts.

My invention consists in a novel construction of the bodies of wagons and other vehicles, by forming the sides, back, and dash-board of paper, treated with a water-proof material, whereby not only lightness and strength, together with durability under exposure to weather, and facility for varnishing or polishing, are secured, but said parts are not liable to warp or to chip or break, and the same may be got up cheap, and be put together with or without supporting framework.

Referring to the accompanying drawing,

*a a* represent the sides, *b*, the back, and *c*, the dash-board, all made up of hard-pressed paper or paper-pulp, treated with any suitable water-proof material, and put together by dovetailing and screws, or otherwise. The bottom and seat or seats of the vehicle may also, if desired, be made of similar material, treated in like manner, or they may be constructed of different material or materials.

A good water-proof solution for treating the sides, back, and dash-board, made of paper, as described, and cut to any required form and size, may be made

by mixing together the following ingredients, in or about the proportions specified, viz:

Five (5) gallons linseed-oil.

Twenty-five (25) pounds tar-pitch.

Five (5) pounds rosin.

Half of one ( $\frac{1}{2}$ ) gallon spirits of turpentine.

The whole mass to be heated sufficiently to dissolve the rosin and forming a liquid solution, which may be applied to the paper parts of the body herein named, either with the brush, by dipping, or otherwise.

After the solution has been applied, the paper should be dried at a temperature of from 140° to 150° Fahrenheit.

By this improvement, all the advantages hereinbefore specified are secured, namely, cheapness, lightness, strength, and durability under exposure to the weather, with an enlarged capacity for taking a high polish, and freedom from warping, breaking, or chipping; also, whereby the dash-board presents a smoother and neater appearance than one made of leather stretched on an iron frame, and is greatly superior to a wooden one. The dash-board also being made of the same material as the sides and back, the manufacture of the body of the vehicle is greatly facilitated, and a lightness and strength secured for the whole skeleton.

What is here claimed, and desired to be secured by Letters Patent, is—

A wagon or vehicle-body, having its sides, back, and dash-board made of paper, treated with water-proof material, substantially as specified.

J. W. JARBOE.

Witnesses:

HENRY T. BROWN,

EDWD. ADAMS.